

UNITED STATES PATENT OFFICE.

361,999

ERNEST F. GRETER AND CHARLES MOSHER, OF SOUTH BEND, INDIANA.

PROCESS OF TREATING RAW HIDES.

SPECIFICATION forming part of Letters Patent No. 361,999, dated April 26, 1887.

Application filed May 25, 1886. Serial No. 203,244. (S. specimens.)

8-94.18

To all whom it may concern:

Be it known that we, ERNEST F. GRETER and CHARLES MOSHER, of South Bend, in the county of St. Joseph and State of Indiana, have invented certain new and useful Improvements in Processes for Treating Raw Hides; and we do hereby declare that the following is a full, clear, and exact description thereof.

This invention is an improved process of 10 treating raw hide to render the same hard, elastic, and water-proof; and it consists in the steps hereinafter described, and pointed out in the appended claims.

As the product of the process differs in some 15 essential points from anything of the kind produced before, it is also included in the invention and embraced in the claims.

The process is as follows: The hide, being properly washed and cleaned in the ordinary 20 manner to remove dirt, is treated with lime at a temperature of not over 90° Fahrenheit to denude it of hair. The hair being thus removed, the hide is stretched and nearly dried. It is then disinfected by placing it in a bath 25 of bromo-chloralum and water, the proportions of which in the bath are about one gallon of bromo-chloralum to twenty gallons of water, or a bath may be used composed of one ounce of carbolic-acid crystals or two ounces of ordinary commercial carbolic acid to the gallon of 30 water. We prefer, however, the first-described bath. The hide is left in this disinfecting-bath for about six hours, according to the state or condition of the hide, the time of immersion 35 varying in length for "sweet" or fresh hides and those that are old or tainted. After immersion in this bath for a proper length of time, the hide is removed and passed between rollers to wring it, and again stretched and 40 nearly dried. The hide is then immersed in a bath of the soluble silicate of soda for about eight hours, or until it is saturated with the silicate. This soda-bath is made in about the proportion of one gallon of commercial silicate 45 of soda to two gallons of lukewarm water. It is then again nearly dried and submitted to the rollers, so as to solidify it by pressure, after which the drying is completed at a temperature of not over 112° Fahrenheit. The 50 dried hide is now passed between pressure-rollers, so as to reduce it to one uniform thick-

ness. Then it is varnished with suitable varnish, shellac, or asphaltum.

The rollers used in wringing out the hides and pressing them to a uniform thickness may 55 be of any suitable kind—such, for instance, as the rolling-machine used by tinsmiths to reduce metal to different thicknesses. The rolls proper may be made of wood, rubber, metal, or any suitable material, as they form no part 60 of the invention, and various other means may be employed for wringing the hides and for reducing them—such, for example, as hydraulic presses, a roll moving over a plane surface, drop or trip hammers, or pounding by 65 hand, and many other ways known to those skilled in the art.

The process being thus completed, it will be found that the hide has become essentially a new material, the mechanical treatment causing it to become hard and elastic, and the absorbed silicate and varnish entangled in its fibers by the pressure and not removable therefrom rendering it water-proof.

The power of the hide to resist the action of 75 water is increased to some extent by giving it a coating of a suitable varnish, and by this means we can vary the color of our product as desired, and at the same time impart to its surface a finished appearance.

80 This product is well adapted for the manufacture of surgical splints and other articles, and it is also a good substitute for whalebone.

Having described our invention, we claim—

1. The herein-described process for treating 85 raw hide to render it hard, elastic, and water-proof, which process consists in washing the hide, treating it with lime at a temperature not above 90° Fahrenheit to remove the hair, stretching and nearly drying it, immersing it 90 in a bath of dilute carbolic acid or bromo-chloralum for disinfecting purposes, passing it between rollers under pressure, and again stretching and nearly drying it, immersing it in a bath of the soluble silicate of soda until it 95 is saturated therewith, then partly drying it and subjecting it again to roller-pressure to solidify it, then completing the drying of it at a temperature not over 112° Fahrenheit, then varnishing it, and passing it again between 100 the rollers until it is reduced to a uniform thickness.

2. The herein-described process for treating raw hides to render them hard, elastic, and water-proof, which process consists in subjecting a hide after partial drying to a bath of dilute disinfectant—such as bromo-chloralum or carbolic acid—passing it between rollers to facilitate drying, and stretching and nearly drying it, immersing it in a bath of a soluble silicate—such as silicate of soda—until saturated therewith, then partly drying it, then varnishing it, subjecting it to pressure to solidify, then completely drying it at a temperature not to exceed 112° Fahrenheit, and

passing through rollers to render it uniform in thickness, then varnishing it to give it 15 color and a finished appearance, substantially as set forth.

In testimony that we claim the foregoing as our own we affix our signatures in presence of two witnesses.

ERNEST F. GRETHER.  
CHARLES MOSHER.

Witnesses:

JAMES DU SHANE,  
CHAS. W. WILEY.